

# United States Patent Office.

SANFORD A. HICKEL, OF SPENCER, WEST VIRGINIA.

*Letters Patent No. 71,485, dated November 26, 1867.*

## IMPROVED ENAMEL FOR LEATHER.

The Schedule referred to in these Letters Patent and making part of the same.

TO ALL WHOM IT MAY CONCERN:

Be it known that I, SANFORD A. HICKEL, of the town of Spencer, in the county of Roane, and State of West Virginia, have invented a new and improved Enamel for Finishing Leather; and I do hereby declare that the following is a full description of the same, as composed of the following-named ingredients; (a specimen of the said ingredients and the composition is herewith presented:)

The nature of my invention consists in combining one (1) gallon of alcohol; one and a half ( $1\frac{1}{2}$ ) pound gum-shellac, or any other water-proof gum; three-fourths ( $\frac{3}{4}$ ) of a pound of Burgundy pitch, or any other extract of rosin or turpentine; one ounce of camphor; and dissolve these together. Two (2) ounces gum-copal; two (2) ounces rosin; pulverize these together, and dissolve them in one-half ( $\frac{1}{2}$ ) pint of turpentine. After this is dissolved, add it to the first compound, composed, as above, of one gallon of alcohol, one and a half pound gum-shellac, or any other water-proof gum, three-fourths of a pound of Burgundy pitch, or any other extract of rosin, and one ounce of camphor. Then add to this compound three (3) ounces of clarified lamp-black or the same quantity of ivory-black.

This makes a thorough water-proof finish, which neither change of weather, water, nor oil will affect the body of. The finish is elastic, and will not fracture, and may be applied to many other purposes besides the finishing of leather, as, for instance, to finishing and enamelling wood, iron, steel, and cloth. It keeps the leather soft and pliable, and therefore durable, and makes a fine and durable lustre.

In using the enamel, the stock must first be thoroughly cleaned and dried; the enamel may then be applied with a sponge or any other soft substance, and it will dry as quickly as any ordinary finish.

What I claim as my invention, and desire to secure by Letters Patent, is—

The combination of the above materials or ingredients in the proportions named, and the resulting compound; the improved enamel finish, and the application of the same to leather, wood, iron, steel, and cloth.

SANFORD A. HICKEL.

Witnesses:

SAMUEL YOUNG,

JOHN A. HURLEY.